

## UNITED STATES PATENT OFFICE

1,947,219

## TREATMENT OF MOTOR FUEL

Paul I. Murrill, Norwalk, Conn., assignor to R. T. Vanderbilt Company, Incorporated, New York, N. Y., a corporation of New York

No Drawing. Application May 21, 1931  
Serial No. 539,134

15 Claims. (Cl. 44—9)

This invention relates to a new and improved treatment of motor fuel. It includes both the method of treatment and the product obtained.

Difficulty has been experienced with the formation of gum in motor fuels. A gasoline which is pure distillate, free from non-volatile matter, may, on evaporation, form a deposit of gum. This is particularly true of cracked gasolines and more particularly of gasolines produced by cracking at high temperatures. Gasolines produced by cracking petroleum oil in the vapor phase are particularly bad from the standpoint of gum formation. The formation of gum apparently is due to the oxidation of unsaturated constituents of the gasoline. The pure gasoline distillate contains "potential gum" which, on standing, forms actual gum.

This invention relates to the treatment of motor fuels to prevent or retard or inhibit the formation of gum, and particularly it relates to the treatment of motor fuels containing gum-forming unsaturated constituents produced by the cracking of petroleum compounds. More particularly the invention relates to the treatment of motor fuels containing gum-forming unsaturated constituents produced by cracking petroleum oil at a high temperature, e. g. at a temperature of at least 300° C.

According to this invention a small amount of an aromatic di-secondary diamine is added to a freshly distilled gasoline which contains gum-forming unsaturated constituents to delay or prevent the formation of objectionable amounts of gum. In general from two to ten milligrams per one hundred cubic centimeters of gasoline gives good results but larger or smaller amounts of the di-secondary diamine may be used without departing from the scope of this invention. The motor fuels of this invention may contain in addition to gasoline, benzol or other saturated compounds, anti-knock compounds, etc., and the di-secondary diamine may be added to the gasoline before or after blending with the other constituents.

Compounds which have been found effective include the following di-secondary diamines: s-diphenyl-benzidine, and diaryl meta-arylene diamines, e. g. s-diphenyl-m-phenylene diamine, s-di-beta-naphthyl-m-phenylene diamine, and diaryl para-arylene diamines, e. g. s-di-alpha-naphthyl-p-phenylene diamine, s-di-beta-naphthyl-m-phenylene diamine, s-diphenyl-p-phenylene diamine, s-diorthotolyl-p-phenylene diamine, and s-diparatolyl-p-phenylene diamine.

Gasoline is prepared by a variety of methods

and the effectiveness of the various di-secondary diamines varies somewhat with different gasolines. I have obtained positive results with both gasolines produced by cracking in the liquid phase and gasolines produced by cracking in the vapor phase. Results obtained thus far indicate that the diaryl para-arylene diamines, more particularly the ditolyl para-arylene diamines, are generally more effective in prolonging the period before objectionable gum formation sets in than other di-secondary diamines, and this is particularly true with gasolines produced by cracking in the vapor phase. For this purpose I prefer to use s-di-phenyl-p-phenylene diamine, s-diorthotolyl-p-phenylene diamine or s-di-paratolyl-p-phenylene diamine. These are more soluble than s-di-alpha-naphthyl-p-phenylene diamine and s-di-beta-naphthyl-p-phenylene diamine and are preferred for this reason.

This application is in part a continuation of my application Serial No. 491,817, filed October 28, 1930.

I claim:

1. The process of treating cracked gasoline, which comprises mixing therewith before the formation of any substantial amount of gum in the gasoline, a diaryl arylene diamine in an amount sufficient to inhibit gum formation. 80

2. The process of treating cracked gasoline, which comprises mixing therewith before the formation of any substantial amount of gum in the gasoline, a ditolyl arylene diamine in an amount sufficient to inhibit gum formation. 85

3. The process of treating cracked gasoline, which comprises mixing therewith before the formation of any substantial amount of gum in the gasoline, a diaryl para-phenylene diamine in an amount sufficient to inhibit gum formation. 90

4. A motor fuel comprising cracked gasoline and a diaryl arylene diamine in an amount sufficient to inhibit gum formation. 95

5. A motor fuel comprising cracked gasoline and a ditolyl para-phenylene diamine in an amount sufficient to inhibit gum formation.

6. A motor fuel comprising cracked gasoline which contains gum-forming constituents produced by the cracking of petroleum compounds and a ditolyl arylene diamine in an amount sufficient to inhibit gum formation. 100

7. A motor fuel comprising cracked gasoline which contains gum-forming constituents produced by the cracking of petroleum compounds and a diaryl para-phenylene diamine in an amount sufficient to inhibit gum formation. 105

8. A motor fuel comprising cracked gasoline 110

- containing gum-forming constituents produced by the cracking of petroleum compounds at a high temperature and a diaryl arylene diamine in an amount sufficient to inhibit gum formation.
- 5 9. A motor fuel comprising gum-forming constituents produced by the cracking of petroleum compounds and a compound of the general formula  $RNH_2R_2NHR_1$  where  $R$  and  $R_1$  may be the same or different aromatic radicals and  $R_2$  is an aromatic radical, said compound being present in an amount sufficient to inhibit gum formation.
- 10 10. The process of treating cracked gasoline which comprises mixing therewith before the formation of any substantial amount of gum, diortho-tolyl-p-phenylene diamine in an amount sufficient to inhibit gum formation.
- 15 11. The process of treating cracked gasoline which comprises mixing therewith before the formation of any substantial amount of gum, di-para-tolyl-p-phenylene-diamine in an amount sufficient to inhibit gum formation.
- 20 12. The process of treating cracked gasoline which comprises mixing therewith before the formation of any substantial amount of gum, diphenyl-p-phenylene-diamine in an amount sufficient to inhibit gum formation. 80
13. A motor fuel comprising gum-forming constituents produced by the cracking of petroleum compounds at a high temperature and diortho-tolyl-p-phenylene-diamine in an amount sufficient to inhibit gum formation. 85
14. A motor fuel comprising gum-forming constituents produced by the cracking of petroleum compounds at a high temperature and di-para-tolyl-p-phenylene-diamine in an amount sufficient to inhibit gum formation. 90
15. A motor fuel comprising gum-forming constituents produced by the cracking of petroleum compounds at a high temperature and diphenyl-p-phenylene-diamine in an amount sufficient to inhibit gum formation. 95

PAUL I. MURRILL.

25

100

30

105

35

110

40

115

45

120

50

125

55

130

60

135

65

140

70